

Oct. 18, 1932.

P. C. RIPLEY

1,882,917

METHOD OF MAKING INGOTS

Filed Jan. 27, 1930

FIG. 1



FIG. 2



FIG. 3  
Perry C. Ripley.

Charleston,  
W. Va.

547

11175

## UNITED STATES PATENT OFFICE

PERRY C. RIPLEY, OF CHICAGO, ILLINOIS, ASSIGNOR TO KESTER SOLDER COMPANY, OF CHICAGO, ILLINOIS, A CORPORATION OF ILLINOIS

## METHOD OF MAKING INGOTS

Application filed January 27, 1930. Serial No. 423,898.

This invention relates to a process for forming uniform castings of metal alloys, and more particularly to a process for forming such castings from lead and tin alloys in which the ratio of lead to tin varies from the ratio of such metals in a true eutectic mixture. The invention further contemplates a casting so formed.

If lead and tin are fused together in the approximate ratio of three atomic weights of tin to one of lead and heat extracted from the solution, a point is reached where the solution solidifies en masse. This point is termed the eutectic point and the resulting solid the eutectic. Upon examination, it will be found that the solid is, in some respects, a chemical compound having the empirical formula  $BbSn_3$ . According to many authorities, it is in reality a chemical compound.

This lead-tin solid has a lower melting point than any other solid solution of lead and tin and is the only solid solution of lead and tin which is homogeneous; that is, the only alloy of these metals wherein the lead and tin are, in effect, combined as a chemical compound.

It, therefore, follows that any other alloy of lead and tin is composed of the eutectic of lead and tin together with free or uncombined lead or tin held in suspension in the eutectic. Thus, if a mixture of lead and tin containing these metals in other than the atomic proportions of one lead to three tin be fused and slowly cooled, lead or tin, depending upon which is in excess of the eutectic proportion, will precipitate until the eutectic mixture is reached, when the entire solution will freeze en masse. The resulting solid will contain the eutectic plus free lead or tin distributed non-uniformly throughout the solid. Since most commercial alloys of lead and tin are non-eutectic, it is apparent that such alloys, in most instances, are of non-uniform composition, and, especially, is it generally true that large ingots or similar articles made therefrom are of non-uniform composition and, for that reason, objectionable where uniformity is a desired or a requisite property.

Since the excess of tin or lead over the

eutectic proportion precipitates during the gradual cooling of the fused alloy and tends to settle through the still liquid portions of the alloy mass, the slower the rate of cooling the greater the lack of uniformity in the composition of the resulting solid. If, on the other hand, it were possible to lower the temperature of the entire mass of fused lead and tin from its initial solidifying point to the eutectic point practically instantaneously, the resulting eutectic would entrap the crystals of lead or tin in excess of the eutectic before they could fully precipitate or settle out, and, in that way, a substantially uniform alloy would result containing the lead and tin in the proportions throughout the solidified mass in which they existed in the fused mixture.

While it is not only possible but also rather simple to obtain a rate of cooling approximating the above ideal in forming relatively small castings, it can be appreciated that in the formation of large castings a different problem is presented.

I have, however, devised a process wherein I can form relatively large castings of uniform composition from non-eutectic alloys of lead and tin; that is, alloys containing lead and tin in proportions other than those in which they exist in the eutectic. In general, my process consists in first pouring and rapidly cooling small diameter castings to form ingots of substantially uniform composition and then pouring further quantities of the lead-tin solution over and around a core formed of the relatively small ingots in a large jacketed mold, whereby such ingots extract heat from the solution in the central portion of the mold, the solution in the outer portions of the mold being cooled by external means, as by water or the like. In this way, a rapid freezing of the solution is obtained, the net result being a bonding together of the smaller ingots by the solution with the formation of a large ingot having a substantially uniform composition.

It is, accordingly, an object of this invention to provide a process for forming relatively large ingots of a uniform composition throughout from a non-eutectic alloy.

It is a further object of this invention to provide a process for rapidly extracting heat from a lead-tin solution by means of cores formed of small bodies of a uniform composition lead-tin alloy containing the lead and tin in the same proportions as exist in the lead-tin solution.

It is a further object of this invention to provide a relatively large casting of a non-eutectic lead-tin alloy having a substantially uniform composition throughout its mass.

Other and further important objects will become apparent from the following description and appended claims.

My invention is best described in connection with the accompanying drawing in which a preferred embodiment of it is shown.

Figure 1 is a top view of the device showing several molds surrounded by cooling jackets.

Figure 2 is a section taken along the line II-II of Figure 1 with certain parts shown in elevation.

Molds 1, 2, 3, 4, and 5 are located within a tank 6 which has a removable base 13. A cooling liquid circulates through the apparatus entering the tank 6 through pipe 7 and leaving it through pipe 8. Within the molds 1, 2, 3, and 4 are small alloy castings 10 surrounded by the molten metal 9. Figure 2 the small alloy casting 10 is shown in elevation in molds 1, 2, and 3 and in section in mold 4. Mold 5 contains a modification in which several small castings 11, are used. In Figure 2, two of these small castings are shown in section and the center one in elevation.

The molds are preferably arranged on the arc of a circle II-II since this arrangement makes it convenient to pour the metal from a large ladle or pot which is supported from a central axis in such a manner that it may be swung along this arc thereby bringing it into position over each mold for pouring.

According to my invention, I first fuse a mixture of lead and tin to form a solution containing these metals in the proportions desired in the finished casting. For instance, in the formation of ingots to be used in dies for making solder wire in which field this invention has great utility, lead and tin are melted together to form a solution containing approximately 60% of tin and 40% of lead by weight. Relatively small diameter ingots are then formed from this solution by casting the solution into tapered molds of any suitable length and of about 1½ to about 2 inches in diameter, said molds being surrounded by a water jacket or similar cooling means. Due to the relatively small diameter of the molds, an almost instantaneous freezing and solidification of the entire content of each mold is effected, with the result that the excess lead in the solution over the atomic ratio expressed by the eutectic formula PbSn<sub>3</sub> is entrapped

in and uniformly distributed throughout the resulting ingots.

These ingots 10 are then removed from the molds, the removal being promoted by the taper of the molds.

Relatively large diameter ingots represented by both portions 9 and 10 having a weight say, 150 lbs. or more, are then produced by employing the small ingots in the following manner

A number of the relatively small diameter ingots 10 or 11 of uniform composition are grouped at or near the central axis of a large diameter water-cooled mold 1, 2, 3, 4 or 5 of approximately the same height as said smaller diameter ingots. A further quantity of said lead-tin solution is then poured into the mold over and around said smaller ingots to completely fill the voids around and between the small ingots. The smaller ingots rapidly extract heat from the solution coming into contact therewith, whereby that portion of the solution is quickly solidified, thus binding the smaller ingots together. Simultaneously, that part of the solution contacting the periphery of the mold is rapidly frozen by the water or other mold cooling medium, so that the entire body of solution is converted into an homogeneous ingot. Because of the rapidity with which the heat is extracted from the solution, the resulting ingots will be of substantially uniform composition, the excess of lead over the eutectic being distributed throughout the ingots.

The following comparative data obtained from experiments performed on 150-lb. ingots of lead-tin alloys, cast from solutions containing approximately 60% tin and 40% lead by weight, according to the conventional method and the method of this invention, serve to indicate the great difference in the uniformity of the composition of the ingots resulting from the two processes. Three 150-lb. ingots were prepared first by casting a molten mixture of 60% tin and 40% lead into molds and then three other 150-lb. ingots were prepared by my process.

Each of the three ingots prepared by the conventional method was then extruded through dies in the form of wire solder. Upon analysis of the wire solder as the extrusion progressed, the tin content showed a maximum variation in the case of one ingot of 5.24%, in another 3.53% and in the third 3.04%. The average maximum variation in the composition of the three ingots throughout their respective masses was, therefore, 3.97%.

The tin content of the wire extruded from the three ingots prepared in accordance with my invention was then progressively analyzed. In one ingot there was a maximum variation of 0.74%, in another 0.61% and in the last 0.54%, or an average maximum variation of 0.61%.

It can thus be appreciated that my method

constitutes a decided improvement over the methods now in use in this art, since it permits the casting of relatively large ingots of substantially uniform composition. The use of larger ingots obviously makes for greater economies in production in permitting the use of larger capacity machines for extruding the metal alloys in the form of solder wire or the like. Further, the substantial uniformity of composition throughout the length of 10 solder wire produced from the large ingots of my invention makes for uniform soldering results.

While, in the preferred method of carrying out my process, a plurality of small diameter ingots are bonded together in forming a relatively large diameter ingot, it is to be understood that a single small diameter ingot may be employed to form an ingot of a slightly larger diameter, and this, in turn, 20 used to build up a still larger ingot, until an ingot of desired size is obtained.

It should also be borne in mind that, while my disclosure particularly deals with the formation of ingots from an alloy containing 25 by weight 60% tin and 40% lead, yet this is not to be construed as a limitation, as castings of uniform composition of other lead-tin alloys, as well as alloys of other metals, can be 30 efficaciously made by my method.

Other changes may also be made in the method disclosed without departing from the spirit of my invention and, accordingly, I do not propose to limit the invention claimed herein other than as necessitated by the prior 35 art.

I claim as my invention:

1. The process of preparing a relatively large diameter ingot of substantially uniform composition throughout from an alloy 40 containing by weight approximately 60% of tin and 40% of lead, which comprises casting a solution containing lead and tin in the ratio of 60% tin and 40% lead about a core 45 comprising a relatively small tin-lead alloy ingot having a diameter not greater than about two inches and being of uniform composition containing 60% of tin and 40% of lead whereby to effect a rapid extraction of 50 heat from that portion of the solution contacting said small ingot and simultaneously effecting a conduction of heat from the remainder of the solution whereby a rapid freezing of the entire mass of solution is 55 obtained.

2. The process of preparing a relatively large diameter ingot of substantially uniform composition from a non-eutectic lead-tin alloy, which comprises casting a solution 60 containing lead and tin in a ratio other than that in the eutectic over and around a plurality of relatively small lead-tin alloy ingots each having a diameter not greater than about two inches and being of uniform composition in 65 which the lead and tin are in the same ratio.

as in said solution to thereby effect a rapid extraction of heat from that portion of the solution contacting said small ingots and a bonding together of said ingots and simultaneously effecting a conduction of heat from the remainder of the solution, whereby a rapid freezing of the entire mass of solution is obtained.

3. As a new article of manufacture, a non-eutectic tin-lead alloy ingot having a diameter greater than two inches and having a substantially uniform composition throughout its mass, said uniform composition having a maximum variation of less than .74%.

In testimony whereof I have hereunto subscribed my name at Chicago, Cook County, Illinois.

PERRY C. RIPLEY.

85

90

95

100

105

110

115

120

125

130